

**[54] ELECTROPLATING CHROMIUM AND CHROMIUM ALLOYS**

[76] Inventors: **John Cooper Crowther**, 20 St. Leonard's Oval; **Roger Frederick Ashpole**, 62 Beckwith Rd., both of Harrogate, England

[22] Filed: **Feb. 22, 1972**

[21] Appl. No.: **228,083**

**[30] Foreign Application Priority Data**

Feb. 23, 1971 Great Britain ..... 05270/71

[52] U.S. Cl. .... **204/43 R**, 204/51

[51] Int. Cl. .... **C23b 5/32**, C23b 5/06

[58] Field of Search..... 204/294, 51, 105 R, 43 R

**[56] References Cited****UNITED STATES PATENTS**

2,693,444 11/1954 Snavely et al..... 204/51 X  
2,822,326 2/1958 Safranek ..... 204/51 X

**FOREIGN PATENTS OR APPLICATIONS**

7,005,999 10/1970 Netherlands..... 204/51  
1,144,913 3/1969 Great Britain..... 204/51

**OTHER PUBLICATIONS**

C. J. Brockman, "Electrochemistry-Principles and Practice," pp. 152-153, (1931). TP255 B7.

*Primary Examiner*—G. L. Kaplan  
*Attorney, Agent, or Firm*—Herbert H. Goodman

[57]

**ABSTRACT**

An improved process for electroplating chromium and chromium alloys from a substantially aqueous electrolyte containing trivalent chromium ions as the source of chromium and containing oxyanions (preferably sulphate ions) as the major anion component. The improvement comprises incorporating into said electrolyte chlorine ions in an amount of at least 0.1 gram ions per litre or bromine ions in an amount of at least 0.05 grams ions per litre, and a nitrogen compound selected from the group consisting of ammonium compounds, hydroxylamine, hydrazine, urea, aliphatic amines and heterocyclic amines; and utilizing a carbon anode and electroplating chromium from said electrolyte with said carbon anode immersed in said electrolyte. The chlorine ion is preferred and the use of ammonium compounds is preferred.

**21 Claims, No Drawings**

## ELECTROPLATING CHROMIUM AND CHROMIUM ALLOYS

Known electroplating processes employ a variety of anions in the electrolyte notable among which are halogen anions and oxygen-containing anions, such as sulphate.

With the oxygen-containing anions presently used oxygen is liberated at an inert anode. If the latter is of carbon it is attacked by the oxygen with consequent erosion. Also particles of carbon are produced which may deposit on the cathode causing faults in the plated article.

If chlorine or bromine anions are used then the free halogen is liberated at the anode in preference to oxygen. However, the halogen brings its own problems and in any case the plated surface produced is not necessarily equivalent to that obtainable using an oxygen containing anion.

The present invention provides an electroplating process employing a carbon anode and an electrolyte wherein a major proportion of the anions are oxy anions and which further comprises chlorine or bromine ions and a dissolved nitrogen-containing compound which will react with chlorine or bromine in aqueous medium to form nitrogen. By use of such an electrolyte the advantageous plating characteristics afforded by use of oxygen containing anions are substantially retained whilst the gaseous products of the electrolysis evolved in the vicinity of the anode consist wholly or in part of nitrogen instead of oxygen, thus lessening or preventing the erosion of the carbon anode.

It is thought that the operative principle in the novel process is obtaining an electrolyte in which the species having the lowest discharge potential of all anionic species present, including hydroxyl ion, is chlorine or bromine ion. These ions tend therefore to be preferentially discharged during the electrolysis, giving free halogen which then reacts with the nitrogen-containing compound to generate nitrogen. Surprisingly, however, only a small proportion of the nitrogen-containing compound and halogen ions relative to the main oxygen containing anion need to be present in order to make a substantial change in the nature of the gas evolved near the anode from oxygen to nitrogen.

The necessary concentrations of halogen ion and nitrogen-containing compound employed in the novel process will depend upon the overall characteristics of the system rendering it vulnerable to the maleficent effects of oxygen and upon the degree of the consequent impairment which can be tolerated. Clearly anodes whose physical characteristics give them a comparatively high resistance to oxygen attack may be used without disadvantage with electrolytes having lower halide ions and/or nitrogen compound concentrations than would be suitable for less resistant anodes. Also decreasing the anode size and increasing the current density in a given system will make for increased oxygen attack of the electrode. It is preferred that where chlorine ions are employed in the electrolyte they are present in a concentration of at least 0.1 gram:ions per litre, with bromine the preferred minimum is 0.05 gram ions per litre although in both cases concentrations down to as little as 0.01 gram ions per litre may have beneficial effects. The upper limits of concentration of halogen ion are not critical and in many cases will be determined by considerations of solubility, bearing in

mind the need to have enough of the main oxygen-containing ion present in the electroplating system. However we have noticed that in the general case bromine ion tends to reach its maximum effectiveness at concentrations of 0.1 to 0.2 gram ions per litre and chlorine ion at 1.0 to 1.5 gram ions per litre.

The concentration of nitrogen containing compound is not in general critical although it is desirably at least as great as that of the halogen ion and will normally be from one half to twice, e.g. from one to one-and-a-half times that concentration. The upper limit of effectiveness of nitrogen-containing compounds appears to be reached at concentrations of about 3 to 5 molar, e.g. 4 molar.

However, it will not normally be desirable to employ amounts of nitrogen-containing compounds greater than ten percent by weight on the water present since this may unacceptably reduce the solubilities of the metal electroplating salts which generally require the use of substantially aqueous electrolyte solutions.

A convenient way of adding a nitrogen-containing compound and a source of halogen ions is to add a halide of a nitrogen-containing base which has the above-mentioned characteristic of reacting with halogen in an aqueous medium to form nitrogen. If the nitrogenous compound is not a halide salt e.g. if it is urea, the source of halogen ions will normally be the hydrogen halide or an alkali metal halide.

While bromides may also be used in carrying out the invention, the halide which will normally be used is the chloride, and the subsequent description will for the sake of simplicity refer only to chlorides.

When, in accordance with the invention, a source of chlorine ions and a nitrogen-containing compound as defined above is present we believe that the anode reaction proceeds in two stages: first the evolution of chlorine and second the reaction of this chlorine with the nitrogenous compound, although some chlorine may escape in the anodic gas, especially that generated at the top of the anode which has less chance of reaction with the nitrogenous compound in the bulk of the solution. The preferred nitrogenous compounds are ammonium salts and we believe that in that case the second stage of the anode reaction is as follows:



Since the chlorine ion is substantially regenerated in the solution, only the nitrogen-containing compound needs to be replenished. If the latter is a base, it partially neutralises the HCl generated by the reaction and thus tends to maintain the pH of the bath.

The preferred nitrogen-containing compounds are ammonium compounds such as ammonium chloride and sulphate. Also suitable are hydroxylamine, hydrazine, urea and methylamine. Other substances which may be used include aliphatic amides in general including formamide; aliphatic amines in general including methylamine and heterocyclic amines including piperidine. In general it is preferred that the nitrogen-containing compounds comprise not more than five, more preferably not more than four carbon atoms per molecule.

With some nitrogen-containing compounds, e.g. urea, carbon dioxide is evolved together with nitrogen and performs a like function in militating against oxygen attack on the anode.

The invention may be used to special advantage where the anion of the plating bath is  $\text{SO}_4$ . In addition to reducing or preventing erosion of carbon anodes in processes where these are necessarily used, the invention enables carbon anodes to be substituted for soluble anodes in processes where the latter are normally used. Examples of this latter type of process are the plating of zinc, nickel and copper, using metallic anodes. The use of carbon anodes would be advantageous in certain circumstances in these processes, particularly in the plating of zinc, if the problem of erosion could be overcome.

In particular the invention may be applied to conventional processes using oxygen-containing anions and a non-carbon anode together with a porous diaphragm to separate anode and cathode reactions. In operation the introduction of halogen ion and nitrogen containing compound into the electrolyte may enable the anode to be of carbon and, in many cases, the diaphragm to be removed.

The novel process for chromium plating desirably operates at a pH below 2.5, preferably 2.3, where the halide is chloride, and below 2.6 where the halide is bromide.

The main example of plating process in which the use of carbon anodes is in practice necessary is the plating of chromium or chromium alloys from a trivalent chromium bath not using a diaphragm. This is due to the fact that if an insoluble metal anode (e.g. lead) is used it assists oxidation of the  $\text{Cr}^{3+}$  to  $\text{Cr}^{6+}$  thus spoiling the plating, while if a soluble metal anode other than of chromium is used it causes contamination. If the anode is carbon and the anion in such a bath is  $\text{SO}_4$  the erosion of the carbon anode can be reduced or prevented by means of the invention.

The invention may be applied to baths having the same constitution, apart from the halide addition, as those hitherto used. The plating baths may include conventional electroplating additives such as brightening and levelling agents.

The process may find particular use in chromium plating to give a 'hard' finish. Previous chromium plating processes being trivalent chromium ion have generally been suitable for forming only 'decorative' finished. Preferred processes of the invention are those leading to 'hard' chromium finishes. 'Hard' and 'decorative' chromium finishes are known terms of art as recognized, for example, in British Standard 4641 of 1970. A normal decorative finish might have a thickness of 20 millionths of an inch or less; a hard finish might have a thickness of from  $\frac{1}{2}$  to 30, more usually from one to five, thousandths of an inch.

The invention is illustrated by the following Examples:

#### Example 1

A chromium plating bath made up as follows:

|                  |   |                   |
|------------------|---|-------------------|
| IM Cr 111        | } | as sulphates      |
| 4M $\text{NH}_4$ |   |                   |
| 3 g/l            |   | Boric acid        |
| 50 g/l           |   | Ammonium chloride |

was electrolysed in a non-compartmented cell using a nickel cathode and a carbon anode. After passage of 10 ampere hours per litre of solution, no erosion of the anode material was noted, and a satisfactory deposit of

chromium was obtained. By way of comparison, a similar solution, omitting the ammonium chloride, was similarly electrolysed, and after passage of 10 ampere hours per litre of solution, the carbon anode was badly eroded, and particles of carbon could be filtered out of the electrolyte. The deposit of chromium contained inclusions of carbon which resulted in an unsatisfactory coating.

#### Example 2:

To a 100 litre electrowinning bath containing 196 grams chromium sulphate per litre (Bath A) one equiv. (53.5gms) per litre of ammonium chloride was added (Bath B). The solution was electrolysed at 40°C at 10 amps/dm<sup>2</sup> in a non-diaphragm cell using a carbon anode (5dm<sup>2</sup> area) and a stainless steel cathode (5dm<sup>2</sup> area) spaced at 3cm from each other. After the passage of 1,000 amperehours no anode attack was noted. Nitrogen evolution was the main reaction at the anode, although a trace of chlorine could be smelt occasionally. The rate of loss of ammonium ion was found to be close to that predicted by the equation on page 5 hereinbefore, and assuming  $\text{Cl}_2$  to be the primary anode product.

A similar experiment (C) using Bath A without addition of ammonium chloride showed severe anode attack after 1,000 ampere-hours, the main anodic products being carbon dioxide (from the anode) and oxygen.

A similar experiment (D) using Bath A with addition of one equiv. (66gm.) ammonium sulphate per litre instead of ammonium chloride showed severe anode attack after 1,000 ampere hours, the main anodic products being again carbon dioxide and oxygen.

A similar experiment (E) using Bath A with addition of one equiv. (58.5gm) of sodium chloride per litre instead of ammonium, showed slight anode attack after 1,000 ampere-hours, the main anodic products being chlorine gas and oxygen.

Chromium metal of 98.8 percent purity (remainder mainly oxygen) was produced at 30 percent current efficiency from Bath B. The voltage required across the cell was 20 percent lower than in a similar experiment using the same solution in a cell containing a microporous diaphragm, the anolyte being 30 percent sulphuric acid and the anode being 1 percent Ag/Pb alloy.

Cost of electrical power was thus 20 percent lower than in the prior art diaphragm cell, also operated at 30 percent current efficiency.

The design of the cell was also simplified, in that microporous diaphragms were not necessary, and a separate anolyte system was not required.

#### EXAMPLE 3:

In a plating bath (F) made up as follows:

|                    |     |                               |
|--------------------|-----|-------------------------------|
| Chromic sulphate   | 196 | gms. per litre<br>of solution |
| Ammonium sulphate  | 264 |                               |
| Boric acid         | 3   |                               |
| Dimethyl formamide | 80  |                               |

articles were chromium plated in a non-diaphragm cell, using a carbon anode. After the passage of 10 ampere hours per litre of solution it was noted that the deposit of chromium metal on the articles to be plated was patchy, containing areas of low coverage. A particle of carbon could usually be found in the centre of each such thin area. Serious anode attack was noted. The in-

sertion of a microporous diaphragm between anode and cathode improved the deposit quality, but serious anode erosion was still noted. Continuous filtration of the catholyte, i.e., the solution surrounding the articles to be plated was beneficial. The use of anodes other than carbon, in a non-diaphragm cell, led to the production of hexavalent chromium at the anode; this hexavalent chromium reduced plating rates and led to a dark, non-shiny plating.

A similar solution (G) was made up, replacing one equiv. of ammonium sulphate by one equiv. of ammonium chloride, as follows:

|                    |     |                |
|--------------------|-----|----------------|
| Chromic sulphate   | 196 | gms. per litre |
| Ammonium sulphate  | 198 |                |
| Ammonium chloride  | 54  |                |
| Boric acid         | 3   |                |
| Dimethyl formamide | 80  |                |

This solution was used to chromium plate articles in a non-diaphragm cell, using a carbon anode. After the passage of 10 ampere-hours per litre of solution, bright chromium plate equivalent to that plated from the freshly prepared solution, was still being produced. Inspection of the anode revealed no attack, and filtration of the solution showed no deposit on the filter.

#### EXAMPLE 4:

A solution (H) similar to (G) above except that the 54 gm. of ammonium chloride were replaced by 98 gms. of ammonium bromide (1 mole), was used at pH 2.6, in a similar manner to the procedures of example 3. Satisfactorily bright chromium plating was produced which showed no tendency to deteriorate with time. No hexavalent chromium could be detected in the solution 35 after passage of 10 ampere-hours of current per litre.

We claim:

1. In the process of electroplating chromium and chromium alloys on a cathode from a substantially aqueous acidic electrolyte containing trivalent chromium ions as the source of chromium metal which is electroplated and containing oxyanions as the major anion component, the improvement which consists in: (A) incorporating into said electrolyte at least 0.1 gram ions per litre of halogen ion as chlorine ion or at least 0.05 gram ions per litre of halogen ion as bromine ion, and a nitrogen-containing compound selected from the group consisting of ammonium compounds, hydroxylamine, hydrazine, urea, aliphatic amines and heterocyclic amines; the concentration of said nitrogen-containing compound being at least half that of said halogen ion and not greater than 5 molar and the concentration of said halogen ion being not greater than twice that of said nitrogen-containing compound; the anionic species of said electrolyte with the lowest electrical discharge potential being said chlorine or bromine ions; (B) utilizing a carbon anode and electroplating chromium from said electrolyte with said carbon anode immersed in said electrolyte.

2. A process according to claim 1 wherein said electrolyte contains chlorine ions in a concentration of 1.0 to 1.5 gram ions per litre.

3. A process according to claim 2 wherein said oxyanions are sulphate ions.

4. A process according to claim 3 wherein the concentration of said nitrogen-containing compound in

said electrolyte is from one-half to twice that of said chlorine ions.

5. A process according to claim 4 wherein said nitrogen-containing compound is an ammonium compound.

6. A process according to claim 1 wherein said electrolyte contains bromine ions in a concentration of 0.1 to 0.2 gram ions per litre.

7. A process according to claim 6 wherein said oxyanions are sulphate ions.

8. A process according to claim 7 wherein the concentration of said nitrogen-containing compound in said electrolyte is from one-half to twice that of said bromine ions.

9. A process according to claim 8 wherein said nitrogen-containing compound is an ammonium compound.

10. A process as claimed in claim 1 wherein bromine ions are present in said electrolyte in a concentration of at least 0.05 gram ions per litre.

11. A process as claimed in claim 10 wherein bromine ions are present in said electrolyte in a concentration of from 0.05 to 0.1 gram ions per litre.

12. A process as claimed in claim 1 wherein the concentration of nitrogen-containing compound is less than 10 per cent by weight in the water present.

13. A process according to claim 1 wherein said nitrogen-containing compound is an ammonium compound.

14. A process according to claim 1 wherein said oxyanions are sulphate ions.

15. A process according to claim 1 wherein the concentration of said nitrogen-containing compounds in said electrolyte is from one-half to twice that of said halogen ion.

16. A process according to claim 1 wherein the concentration of said nitrogen-containing compound in said electrolyte is from 3 to 5 molar.

17. In the process of electroplating chromium and chromium alloys on a cathode from a substantially aqueous acidic electrolyte containing trivalent chromium ions as the source of chromium which is electroplated and sulphate ions as the major anion component, the improvement which consists in: (A) incorporating into said electrolyte at least 0.1 gram ions per litre of halogen ion as chlorine ion or at least 0.05 gram ions per litre of halogen ion as bromine ion and an ammonium compound; the concentration of said ammonium compound being at least half that of said halogen ion and not greater than 5 molar and the concentration of said halogen ion being not greater than twice that of said ammonium compound, the anionic species of said electrolyte with the lowest electrical discharge potential being said halogen ions; (B) utilizing a carbon anode and electroplating chromium from said electrolyte with said carbon anode immersed in said electrolyte.

18. A process according to claim 17 wherein said halogen ion is chlorine ion and the pH of said electrolyte is below 2.3.

19. A process according to claim 18 wherein said chlorine ion is present in a concentration of from 1.0 to 1.5 gram ions per litre and said ammonium compound is present in a concentration of from 3 to 5 molar.

**20.** A process according to claim 17 wherein said halogen ion is bromine ion and the pH of said electrolyte is below 2.6.

**21.** A process according to claim 20 wherein said bromine ion is present in a concentration of from 0.1

to 0.2 gram ions per litre and said ammonium compound is present in a concentration of from 3 to 5 molar.

\* \* \* \* \*